

# UNITED STATES PATENT OFFICE.

WILLIAM H. BUELL, OF NEW HAVEN, CONNECTICUT, ASSIGNOR TO WINCHESTER REPEATING ARMS COMPANY, OF NEW HAVEN, CONNECTICUT, A CORPORATION OF CONNECTICUT.

## CARTRIDGE-CASING.

1,205,942.

Specification of Letters Patent. Patented Nov. 21, 1916.

No Drawing.

Application filed April 8, 1915. Serial No. 20,087.

To all whom it may concern:

Be it known that I, WILLIAM H. BUELL, a citizen of the United States, and a resident of New Haven, county of New Haven, State 5 of Connecticut, have invented certain new and useful Improvements in Cartridge-Casings, of which the following is a specification.

My invention relates to cartridges for fire 10 arms, especially small arms, and has for its object to produce durable and reliable ferrous metal cartridge casings such as primers and cartridge cases of both the rim fire and the center fire type.

15 It is well known to those skilled in the art, that center fire ammunition is today made by first forming a cup from a sheet of metal and subsequently drawing it by successive drawing to the desired shape.

20 The metal in the head of the shell is formed to the proper shape and thickness and provided with an indentation for the purpose of receiving the primer.

Rim fire ammunition is of the so-called 25 folded type. The head of the shell is provided with a circular cavity or recess; in other words it is formed into an outwardly projecting annular, hollow rim. This circular cavity or hollow annular rim is for the 30 purpose of receiving the priming compound. Heretofore, according to the development of the art, it has been necessary in the case of rim fire ammunition to provide a cartridge made of brass containing the mini-

35 mum amount of zinc consistent with the production of sufficient stiffness, wherever priming mixtures containing fulminate of mercury or mercury in any form was to be used. This is for the reason that amalgams 40 are formed between most metals and mercury and with especial ease in the case of zinc alloys so that if a mercury priming mixture was placed in contact in a slightly moist condition with brass containing an

45 appreciable amount of zinc, there would be amalgamation and consequent weakening of the cartridge case. The amount of amalgamation and the degree to which the amalgamation is effective in weakening the cartridge metal is entirely a matter of degree 50 dependent upon the amount of zinc in the alloy, the amount of mercury in the mixture, the condition of the surface of the metal and the temperature and humidity of the 55 place in which the shells are stored. Where

a priming mixture containing no mercury has been used it has been shown that a cartridge case for rim fire ammunition may be made from a brass very rich in zinc. I am aware that attempts have been made to 60 overcome the difficulty of amalgamation in rim fire ammunition so that a mercury primer could be used by inserting various linings both metallic and non-metallic and by various shellacs.

65 In the case of center fire ammunition the priming compound is loaded into a separate primer which may be of brass, high or low in zinc as the case may be, and which primer is in turn inserted into the primer pocket 70 of the cartridge shell so that in the cases where mercuric primers are used, there is no contact of the mercury of the primer with the shell during storage. However, when the cartridge is fired, the mercury left 75 amalgamates with the brass of the shell and the shell will not stand reloading. We have, consequently, the same condition of amalgamation in a brass center fire cartridge as in a rim fire, the extent being merely a matter of degree dependent on the method of 80 manufacture and subsequent handling.

I have discovered that, by the use of a suitable ferrous metal, I am enabled to make 85 satisfactory rim fire and center fire cartridges and primers and that I am thus able to use interchangeably in such casing either a mercuric or non-mercuric priming compound. As it is sometimes desirable for purposes of differentiating in the ignition 90 of a powder to use a non-mercuric primer, I therefore secure the advantage that without previously selecting the shells or carrying shells made from various kinds of metal in stock I am able to prime with either a 95 non-mercuric or mercuric compound according to the requirements of the matter.

I am aware that it has been desirable to 100 make shells from ferrous metals on account of cheapness over copper alloys but there have been serious objections inherent with ferrous metals or alloys, 1st:—that unless specially treated they become oxidized or rusted or otherwise deteriorated due to atmospheric conditions; 2nd:—that there have 105 been certain difficulties in drawing the shells which have been serious and difficult to overcome.

110 Due to the presence of phosphorus, sulfur, manganese, and carbon (approximately .1%

or over) the metal becomes hardened in the operation of drawing or forming the shell and considerable and frequent annealing is required to prevent tearing the stock. The 5 annealing is also complicated especially when appreciable percentages of carbon are present as under such conditions the temperature of annealing and the rate of cooling affect the final temper of the metal and 10 they must be carefully controlled or otherwise even after drawing, the finished shell may be in a hard and brittle condition. On account of these conditions it has never been possible to successfully make and market 15 an iron or steel cartridge. To prevent rust it was impossible to resort to the usual expedient of galvanizing in the case of a primer, or a rim fire or center fire shell because if a mercury mixture were used the 20 zinc coating would be destroyed; and to obviate the necessity of frequent and careful anneals it was necessary to secure properties in the iron or steel not possessed by the brands on the market. Moreover the question 25 of rusting was serious because, if the usual method of galvanizing was employed for protecting the surface of the shell, a fulminate primer could not be used, the marked affinity of zinc for mercury being 30 so great that in the presence of mercury the zinc would practically wash off and leave the iron exposed.

The ferrous metal which I have found to be suitable for cartridge casings consists 35 of nearly pure iron; several brands of steel now upon the market as regular articles of commerce and consisting of approximately 99.95% iron or over can be successfully employed. On drawing to form the shell the 40 metal will not harden to a very marked degree and consequently requires less annealing and less care in controlling the rate of cooling than was required in the cases where

a larger percentage of carbon was present. It may be stated in fact that I have found 45 that such an alloy consisting of almost pure iron approaches very nearly to having the properties of copper and brass as far as elongation, elastic limit and behavior on annealing is concerned, and I have also found 50 that shells made from such an iron are slower to show effects from rust and can be used with or without a mercuric priming charge, as described. Accordingly when I refer in the appended claims to ferrous 55 metal, I mean to define a steel or iron which has the properties and characteristics indicated.

I have further found that by coating as by an electrolytic process or in any other 60 suitable manner, the whole surface of the metal or that part thereof which would come into contact with the priming mixture, with zinc or its equivalent and in turn similarly coating the zinc with copper or any 65 other metal not readily attacked by mercury, a cartridge casing is produced which has special qualities as to resisting rusting action or action due to a mercuric priming charge; such a casing can, of course, be used 70 either with a mercuric or a non-mercuric compound with perfect freedom.

I claim:

A cartridge casing comprising a core of 75 ferrous metal approaching pure iron in composition, and having a coating of zinc deposited thereon, and a coating of copper deposited on such zinc coating, substantially as described.

In testimony whereof I have hereunto set 80 my hand in the presence of two subscribing witnesses.

WILLIAM H. BUELL.

Witnesses:

DANIEL H. VEADER,  
JOHN MCLEAN.